

# UNITED STATES PATENT OFFICE.

RUSSELL M. COOK AND BENNETT GROTTA, OF TAMAQUA, PENNSYLVANIA, ASSIGNEES  
TO ATLAS POWDER COMPANY, OF WILMINGTON, DELAWARE, A CORPORATION OF  
DELAWARE.

## COMPOSITION FOR DETONATORS.

1,385,245.

Specification of Letters Patent.

Patented July 19, 1921.

No Drawing.

Application filed March 31, 1921. Serial No. 457,500.

To all whom it may concern:

Be it known that we, RUSSELL M. COOK and BENNETT GROTTA, citizens of the United States of America, residing at Tamaqua, in the county of Schuylkill and State of Pennsylvania, have invented certain new and useful Improvements in Compositions for Detonators, of which the following is a specification.

10 Our invention relates particularly to an improvement in a composition used for detonating explosive charges, as for example, dynamite, or gelatin, and it has for its object to provide an improved composition of 15 this nature by virtue of which the explosion temperature of the detonating composition may be reduced to a point materially below the explosion temperature of lead azid alone.

20 The heavy metal salts of hydrazoic acid, for example, lead azid, have been proposed alone and in conjunction with other explosives, as a charge for detonators. Lead azid, and most of the heretofore proposed mix-

25 tures of lead azid with other explosives, suffer from the serious disadvantage of having a high explosion temperature. For instance fulminate of mercury explodes upon being heated to 150° C. to 160° C., whereas lead azid explodes at 320° C. to 350° C.

30 The undesirability of this characteristic in a material which is to be exploded by the spit of a fuse, electric spark or like means of ignition, is apparent and has been a recognized drawback to the commercial application of lead azid.

35 We have discovered that a mixture of lead azid, and trinitrophenylmethyl nitroamin, the latter commercially known as tetryl, gives an efficient initiating explosive, the temperature of explosion of which is much lower than that of lead azid itself, and which is much more easily exploded by the spit of a fuse or similar ignition than lead azid alone. The explosion temperature of lead azid alone is 320° C. to 350° C., while the explosion temperature of the lead azid-tetryl mixture is below 250° C.

We have found 80 parts of lead azid to 20 parts of trinitrophenylmethylnitroamin to 50 be an efficient mixture for the purposes recited. The mixture of lead azid and tetryl may be used either as the only charge of a blasting cap or as a priming charge, the main charge consisting of some other explosive or mixture of explosives, as is common in blasting cap manufacture. Trinitrotoluol or trinitrophenylmethylnitroamin or a mixture of trinitrotoluol and trinitrophenylmethylnitroamin as the superimposed composition makes a highly efficient blasting cap having a low explosion temperature.

55 While we have given an example of definite proportions of lead azid and tetryl, we wish it to be understood that any mixture 60 may be used within the limits of 40 parts lead azid and 60 parts tetryl to 95 parts lead azid and 5 parts tetryl. Also a "composition for detonators" is intended to mean any charge used for initiating the detonation of 65 other explosives.

Having described our invention, what we claim is:

1. A blasting cap charge comprising a mixture of lead azid and trinitrophenyl- 75 methylnitroamin.

2. A blasting cap containing a main charge of explosive and a primer charge comprising a mixture of lead azid and trinitrophenyl-methylnitroamin.

3. A blasting cap containing a main charge of trinitrophenylmethylnitroamin and a primer charge comprising a mixture of lead azid and trinitrophenylmethylnitroamin.

4. A blasting cap containing a main charge 85 of explosive on which is superimposed a mixture of lead azid and trinitrophenylmethylnitroamin.

In testimony whereof we affix our signatures in the presence of two witnesses.

RUSSELL M. COOK.  
BENNETT GROTTA.

Witnesses:

GEORGE CHRIST,  
R. C. KNOLL.